

1,567,219

Dec. 29, 1925.

W. C. WILLIAMS

METAL MELTING METHOD

Filed Oct. 13, 1923



## UNITED STATES PATENT OFFICE.

WISTER C. WILLIAMS, OF DECATUR, ILLINOIS, ASSIGNOR TO McLAUGHLIN COAL REDUCTION COMPANY, OF DECATUR, ILLINOIS, A CORPORATION OF SOUTH DAKOTA.

## METAL-MELTING METHOD.

Application filed October 13, 1923. Serial No. 668,319.

To all whom it may concern:

Be it known that I, WISTER C. WILLIAMS, a citizen of the United States, residing at Decatur, in the county of Macon and State 5 of Illinois, have invented certain new and useful Improvements in Metal-Melting Methods, of which the following is a specification.

This invention is concerned with the operation of melting metals such as copper and brass, for example, in the form of billets or scrap; and the primary object of the invention is to provide a new and improved method of performing this operation more 10 expeditiously, at less cost for fuel, and with a much smaller loss by oxidation of the metal than has heretofore been possible.

The invention is illustrated in the accompanying drawing showing a furnace of preferred construction suitable for carrying out the metal melting operations contemplated by the invention.

In the drawing

Fig. 1 is a vertical sectional view of the furnace.

Fig. 2 is a sectional plan on line 2—2 of Fig. 1.

Fig. 3 is a sectional plan on line 3—3 of Fig. 1, and

Fig. 4 is a fragmentary view in elevation of a modified form of discharge flue.

Referring to Figs. 1, 2 and 3 of the drawing, 10 designates a, preferably cylindrical, combustion chamber provided with a removable cover plate 11 formed with an

opening 12 for discharge of products of combustion. Arranged within the combustion chamber and below the opening 12 is a crucible 13 into which the metal billets

40 or scrap are placed, the crucible being supported above the floor of the furnace on blocks 14 which rest on a metal plate 15 covering the clean-out opening 16.

Projecting, preferably tangentially into the side wall of the furnace, through an oblique slot 17 therein is a nozzle or burner 18 designed to introduce into the combustion chamber a mixture, in proper proportions, of pulverized coal and air. The delivery 45 end of the nozzle is flattened at 19 so that the pulverized coal and air enter the fur-

nace through an orifice 20 relatively narrow transversely, but of considerable spread vertically.

In order to carry off the products of combustion issuing through the outlet opening 12, a flue is provided which consists preferably of an upper fixed section 21 and a lower section 22 telescopically arranged in the upper section and supported so as to be capable of being raised and lowered to bring its flared mouth 23 close to or away from the outlet opening 12. The movable section 22 is preferably provided at the top with a spider 24 attached to a wire cable 25 for raising and lowering the device. Preferably the lower section is of somewhat smaller external diameter than the internal diameter of the fixed section 21 so that the lower section may be temporarily swung to one side of the opening 12 for inspecting the melt, the lower edge of the upper section being preferably flared as indicated at 26 to facilitate this movement.

For large furnaces where the crucible must be handled with a crane I prefer to use a flue as shown in Fig. 4. The fixed flue 28 in this construction is offset with respect to the furnace opening 12 and is provided with a swiveled section 29 having two bends 30, 31, whereby a bell mouth 32 is brought over opening 12, part of the weight of the lower section being carried by a chain or cable 33 attached to a revoluble ring 34 whereby the lower section may be swung away from the furnace.

*Operation.*—The crucible is filled with the metal to be melted and placed in the combustion chamber on the blocks 14 and the fuel in combustion is introduced through the burner 18 so that the flames pass circularly or vertically around the crucible and the products of combustion issue from the furnace through opening 12 in the removable cover plate 11 and the take off flue 21, 22. The outlet 12 is relatively small so that the out draft must bend and pass over the top of the crucible which is an open vessel. This construction of the outlet baffles the stream of products of combustion, causing the incombustible ash in the coal to be deposited in the crucible so as to form a

protecting layer or stratum 27 on the upper and otherwise exposed surface of the body of metal 27<sup>a</sup> in the crucible. The result of this is that the oxidation loss has been reduced to a negligible minimum. Ordinarily the loss of metal by oxidation, in operations of the type contemplated, is quite considerable. The melting operation is carried on very expeditiously and the cost of fuel is small. It is possible to use a very low grade of coal provided it is pulverized to the proper degree of fineness. In fact a coal with a considerable ash content is desirable for the reason above noted. The draft may be regulated by raising and lowering the movable lower section 22 of the take-off flue. If desired, the lower section of the flue may be swung to one side of opening 12, without raising the device, for inspection of the melt. When the melting operation is completed the lower flue section is pulled up within the fixed upper flue section 21, the removable top plate of the furnace is taken away, and the crucible grappled and lifted from the furnace. It is an easy matter to remove the slag and ash deposit 27, whereupon the metal is ready to pour into molds. While it is possible to obtain the protection of the metal from oxidation to a considerable extent, at least, by using coal pulverized to the fineness common to a number of fuels of this type now used, for example, when pulverized so that it will pass through a screen having two hundred meshes to the linear inch, the use of fuel as relatively coarse as this in the furnace as described presents difficulty particularly in the matter of slagging and obtaining complete combustion of the coal as to make these fuels practically useless for this operation. At least very much more satisfactory results are obtained by using a fuel, a considerable portion of which is much more finely pulverized than this. Preferably I use a fuel 90% of which, by weight, will pass through a screen having two hundred meshes to the linear inch, while 25% of it, approximately, will pass through the screen having eight hundred meshes to the square inch. The fuel is introduced into the furnace, as is possible on account of its fineness, on an air current of extremely low pressure, for example, a pressure of not more than one-half ounce. The extremely fine fuel burns at the end of the nozzle, the finest particles of slag being apparently vaporized and passing out through the furnace in that form. The progressively larger particles of fuel, the fuel particles being, of course, graduated in size, are consumed as the flame moves away from the nozzle, combustion being complete within a short distance of the nozzle. The result is that the combustion is complete and there is very little slagging or deposit of ash within the furnace. The deposit of incombustibles

takes place as described, on the metal in the crucible as the flame is baffled in passing out of opening 12.

Whatever the correct theory of operation may be, practical use of the furnace has demonstrated that in order to avoid difficulties of a very serious character a fuel must be used of the size described and must be introduced in the furnace as above set forth.

I claim:

1. Method of melting metal which consists in subjecting the metal in an open container to the heat of a pulverized fuel flame directed so that the incombustibles in the flame are precipitated and deposited upon the metal.

2. Method of melting metal which consists in subjecting the metal in an open container to the heat of a pulverized fuel flame directed so that it passes around the container circularly and over the top of the same depositing the incombustibles of the flame upon the metal.

3. Method of melting metal which consists in subjecting the metal in an open container arranged in a confined space to the heat of a pulverized fuel flame directed circularly around said container and issuing out of the space above the container and baffled at its outlet so that it deposits incombustibles on the metal in the container.

4. Method of melting metal which consists in subjecting the metal in an open container to the heat from a vertical pulverized fuel flame which surrounds the container and in rising above the same is constricted so as to bring about deposit of incombustibles upon the metal.

5. Method of melting metal which consists in subjecting the metal in a container to the heat of a flame directed to pass around the container circularly and produced by the combustion of a solid fuel pulverized so that a portion of it at least is fine enough to burn at the end of the fuel nozzle mixed with air at a low pressure just sufficient to carry the fuel into the furnace without producing any appreciable blast.

6. Method of melting metal which consists in subjecting the metal in an open container to the heat of a flame directed to pass around the container circularly and over the top of the same and produced by the combustion of a solid fuel pulverized so that a portion of it at least is fine enough to burn at the end of the fuel nozzle mixed with air at a low pressure just sufficient to carry the fuel into the furnace without producing any appreciable blast.

7. Method of melting metal which consists in subjecting the metal in an open container to the heat of a flame produced by the combustion of a solid fuel pulverized so that substantially one-fourth of it, by weight, is fine enough to pass a screen having 300

meshes to the linear inch and mixed with air at less than one-half ounce pressure per square inch.

8. Method of melting metal which consists in subjecting the metal in an open container to the heat of a flame directed to pass around the container circularly and over the top

of the same and produced by the combustion of a solid fuel pulverized so that substantially one-fourth of it, by weight, is fine enough to pass a screen having 800 meshes to the linear inch and mixed with air at a pressure of less than one-half ounce per square inch.

WISTER C. WILLIAMS.